

|                |                                                                         |                                       |        |
|----------------|-------------------------------------------------------------------------|---------------------------------------|--------|
| [72] Inventors | Keisuke Shiba;<br>Masanao Hinata; Akira Sato, all of<br>Kanagawa, Japan | 2,422,080 6/1947 Collins et al. ....  | 96/104 |
| [21] Appl. No. | 856,487                                                                 | 2,973,264 2/1961 Nys et al. ....      | 96/104 |
| [22] Filed     | Sept. 9, 1969                                                           | 3,255,012 6/1966 Glockner et al. .... | 96/100 |
| [45] Patented  | Nov. 2, 1971                                                            | 3,348,949 10/1967 Bannert et al. .... | 96/104 |
| [73] Assignee  | Fuji Photo Film Co., Ltd.<br>Kanagawa, Japan                            | 3,463,640 8/1969 Ficken et al. ....   | 96/104 |
| [32] Priority  | Sept. 9, 1968                                                           |                                       |        |
| [33]           | Japan                                                                   |                                       |        |
| [31]           | 43/64854                                                                |                                       |        |

[54] **SPECTRALLY SENSITIZED SILVER HALIDE  
PHOTOGRAPHIC EMULSION**  
10 Claims, No Drawings

|                           |                                                                   |
|---------------------------|-------------------------------------------------------------------|
| [52] U.S. Cl.....         | 96/124,<br>96/100, 260/240.6, 260/240.65, 260/240.7,<br>260/240.8 |
| [51] Int. Cl.....         | G03c 1/28,<br>G03c 1/40                                           |
| [50] Field of Search..... | 96/104, 106                                                       |

[56] **References Cited**  
UNITED STATES PATENTS

|                                       |        |
|---------------------------------------|--------|
| 2,052,754 9/1936 Dieterle et al. .... | 96/106 |
|---------------------------------------|--------|

**ABSTRACT:** Photographic silver halide emulsions and color photographic light-sensitive materials containing same, which emulsions comprise at least one benzimidazolocarbocyanine dye combined with at least one pseudocyanine dye containing either a benzothiazole or benzoselenazole nucleus and hydroxy-substituted at the 5-position thereof. The emulsions may optionally contain, in addition a compound containing a benzimidazole nucleus. The emulsions resulting from the above combination of ingredients are green-sensitive emulsions possessing a uniformly high spectrally sensitized sensitivity over a region from 480 to 580  $\mu$  and are not affected adversely by the presence of a color coupler in the emulsion. Further, the above combination of additives do not produce color stain upon development.

SPECTRALLY SENSITIZED SILVER HALIDE  
PHOTOGRAPHIC EMULSION

## BACKGROUND OF THE INVENTION

## Field of the Invention

The present invention relates to spectrally sensitized silver halide photographic emulsions and, more particularly, to supersensitized silver halide photographic emulsions having increased spectral sensitivity in the green-sensitive region.

## Description of the Prior Art

It is well known that spectral sensitizing is one of the techniques for producing silver halide photographic emulsions. The spectral sensitivity obtained is largely influenced by the chemical structure of the sensitizing dyes used, the halogen composition of the silver halide contained in the emulsion, the crystalline system thereof, the extent of the chemical sensitization, the method of the chemical sensitization, the  $pAg$  of the emulsion, the pH thereof, the kind of binder contained in the emulsion, the kind and properties of stabilizers present, the kind and properties of antifogants present, the kinds and properties of the wetting agents employed, and the kinds and properties of hardening agent present.

Moreover, such additives frequently act to lower the spectrally sensitized sensitivity of the emulsion. In particular, in the case of color photographic light-sensitive materials, the chemical structures of the sensitizing dyes and the manner of using them must be specifically selected so that the adverse influences of the colored couplers contained in the emulsions on the spectrally sensitized sensitivity are reduced as much as possible.

Further, some sensitizing dyes are known to impart higher sensitivity when they are used together with other dyes or colorless aromatic compounds having specific chemical structures, as compared with using these dyes individually. This is known as supersensitization. Combinations of compounds which provide supersensitization are required to be very rigidly selected. Thus, it is important to the spectral-sensitizing technique to find combinations of compounds which will coact to provide supersensitization.

Spectral sensitization for the green-sensitive region corresponding to a spectral region of high visual sensitivity is most important for the color reproduction of a color photographic light-sensitive material and the quality of the color image formed thereon. In regard to the spectral sensitization of the green-sensitive region, there is described, e.g., in U.S. Pat. No. 2,701,198, a method wherein a benzimidazolonecarbocyanine dye and a pseudocyanine dye are used. However, when this combination of sensitizers is employed in emulsions of color photographic light-sensitive materials, the spectral sensitizing action is only slightly obtained owing to the adverse influence of a color coupler present together with them. Moreover, although the method disclosed in the above U.S. patent results in a supersensitizing action, the supersensitization and the green sensitivity thus obtained are lower than those obtained by using a combination of, for example, a benzimidazolocarbocyanine dye and a benzoxazolocarbocyanine dye (see Japanese Pat. Publication No. 4936/68).

One reason for the disadvantages of the method of the above U.S. patent is considered to be a harmful inhibiting action occurring during the development process. On the other hand, the method shown in the aforesaid Japanese Pat. Publication No. 4936/68 is accompanied by the disadvantage that, although it may provide a high spectral sensitivity in the green region, contamination with dye remaining after the development procedure (hereinafter called "color stain") is large. Further, the latter method is accompanied by another disadvantage, in that the sensitivity in the region from 500 to 530  $m\mu$ , which is a portion of the shorter wave length, green region, is relatively low.

## SUMMARY OF THE INVENTION

Thus, an object of the present invention is to provide a green-sensitive photographic silver halide emulsion which is not reduced in sensitivity when used in the presence of a color coupler, which provides a uniformly high spectral sensitivity over the region from 480 to 580  $m\mu$ , and which further imparts no color stain after the development procedure.

Another object of the present invention is to provide a color photographic light-sensitive material having, on a support, at least one layer of the aforesaid photographic silver halide emulsion.

The inventors have found that the above-mentioned objects of this invention can be attained by incorporating in a photographic silver halide emulsion at least one of the benzimidazolocarbocyanine dyes represented by the formula



wherein  $Z_1$  and  $Z_2$  each represents nonmetallic atoms necessary to complete the benzimidazole nucleus;  $R_1$  and  $R_2$  each represents an alkyl group, a substituted alkyl group or an allyl group;  $R_3$  and  $R_4$  each represents an alkyl group or a substituted alkyl group, at least one of said groups  $R_3$  and  $R_4$  being a sulfo-substituted alkyl group or a carboxy-substituted alkyl group;  $X_1$  represents an acid anion group; and  $p$  is 1 or 2 and at least one pseudocyanine dye represented by the formula



wherein  $Z_3$  represents nonmetallic atoms necessary to complete the quinoline nucleus;  $Y$  represents a sulfur atom or a selenium atom;  $R_5$  and  $R_6$  each represents an alkyl group or a substituted alkyl group, at least one of said groups  $R_5$  and  $R_6$  being a sulfo-substituted alkyl group or a carboxy-substituted alkyl group;  $A$  represents a hydrogen atom, an alkyl group having one to four carbon atoms, or a halogen atom;  $X_2$  represents an anion; and  $q$  is 1 or 2.

Moreover, as one embodiment of the present invention, it has been found that improved results can be obtained by adding to the photographic silver halide emulsion, together with the aforesaid dyes, at least one of the compounds represented by the following formula



wherein  $Z_4$  represents nonmetallic atoms necessary to complete the benzimidazole nucleus;  $R_7$  represents an alkyl group or a substituted alkyl group and  $Z_5$  represents a phenyl group or a substituted phenyl group.

## DETAILED DESCRIPTION OF THE INVENTION

As the sulfo-substituted alkyl group represented by  $R_3$  or  $R_4$  in formula I, there may be exemplified  $\beta$ -sulfoethyl,  $\gamma$ -sulfoethyl,  $\alpha$ -sulfonyl,  $\gamma$ -hydroxy- $\beta$ -sulfonyl, 2-(3-sulfonylpropoxy)ethyl, 2-[3-(3-sulfonylpropoxy)ethoxy]ethyl and the like. Further, as the carboxy-substituted alkyl group represented by  $R_3$  or  $R_4$ , there may be exemplified  $\beta$ -carboxyethyl,  $\beta$ -carboxypropyl, 2-(2-carboxyethoxy)ethyl and the

like. Moreover, as alkyl groups represented by  $R_3$  and  $R_4$ , there may be exemplified methyl, ethyl, n-propyl and the like. As the substituted-alkyl group, there may be exemplified, besides the aforesaid sulfo-substituted alkyl group and the carboxy-substituted alkyl group,  $\beta$ -hydroxyethyl,  $\beta$ -acetoxyethyl and the like.

Furthermore, as the alkyl group and the substituted alkyl group represented by  $R_1$  and  $R_2$  in formula I, there may be exemplified methyl, ethyl, n-propyl,  $\beta$ -acetoxyethyl, and an alkyl group.

$Z_1$  and  $Z_2$  of the formula represent the atoms necessary to complete the benzimidazole nucleus, as mentioned before, and the benzimidazole nucleus may be halogen, cyano, trifluoromethyl, alkyl-aminosulfonyl, or acetyl-substituted.

The alkyl group or substituted alkyl group represented by  $R_5$  or  $R_6$  in formula II are as set forth above in connection with  $R_3$  and  $R_4$ . At least one of  $R_5$  and  $R_6$  is a substituted alkyl group having either a sulfo group or a carboxyl group as set forth above in connection with  $R_3$  and  $R_4$ .  $Z_3$  in formula II represents the nonmetallic atoms necessary to complete a quinoline nucleus, as mentioned above, and the quinoline nucleus may be substituted by a methyl group, an ethyl group, a hydroxyl group, an alkoxy group or a halogen atom.

$X_1^1$  and  $X_2^1$  in general formulas I and II, respectively, are an anion, such as, a bromine ion, an iodine ion, a thiocyanate ion, an alkylsulfate ion, a perchlorate ion, and a p-toluenesulfonate ion. Also, the case wherein  $p$  is 1 and  $q$  is 1 in these formulas represents the formation of an intramolecular salt.

$R_7$  in general formula III is the alkyl group or the substituted alkyl group as set forth in connection with groups  $R_3$  and  $R_4$  in general formula I. Moreover, as the substituent for the substituted phenyl group shown by group  $Z_5$  in general formula III, there may be illustrated an alkyl group such as a methyl group, an ethyl group, or a propyl group; and alkoxy group such as a methoxy group or an ethoxy group; and a halogen atom such as a chlorine atom or bromine atom.

The feature of the sensitizing dye represented by general formula I is that at least one of  $R_3$  and  $R_4$  is a sulfo-substituted alkyl group or a carboxy substituted alkyl group as mentioned above, which renders the dye reactive for supersensitization by the sensitizing dye represented by general formula II as well as for supersensitization by the compound represented by general formula III.

On the other hand, the feature of the sensitizing dye represented by general formula II is that the benzothiazole or the benzoselenazole nucleus has a hydroxyl group at the 5-position thereof and also at least one of  $R_5$  and  $R_6$  is a sulfo-substituted alkyl group or a carboxyl substituted alkyl group. Most preferably,  $R_6$  is a sulfo-substituted alkyl group.

Sensitizing dyes wherein the benzothiazole or the benzoselenazole nucleus has a hydroxyl group at the 6-position have the drawback that the dye has high desensitizing properties and such dyes tend to form fog upon development. Also, sensitizing dyes having a hydroxyl group on the quinoline nucleus have the disadvantage that such dyes are weak in supersensitizing properties.

Accordingly, it is important that the sensitizing dye have a hydroxyl group at the 5-position of the benzothiazole or benzoselenazole nucleus.

In general, when a pseudocyanine dye having no substituent on the nucleus is substituted by a sulfo-alkyl group at the 5- or 6-position in general formula II, the dye provides hardly any spectral sensitivity. However, when a pseudocyanine dye having a hydroxyl group or a phenyl group at the 5-position of the benzothiazole nucleus or benzoselenazole nucleus is substituted by a sulfo-alkyl group at  $R_5$  or  $R_6$  in the general formula I, the spectral sensitivity obtained is markedly increased.

Furthermore, pseudocyanine dyes having a phenyl group at the 5-position have very weak supersensitizing action to the sensitizing dye represented by general formula I and form severe fog. On the other hand, pseudocyanine dyes having a hydroxyl group at the 5-position provide a strong supersensitizing action.

Since the pseudocyanine dye represented by general formula II and used in the present invention has a sulfo-alkyl or a carboxy-alkyl group and also has a hydroxyl group at the 5-position of the benzothiazole or benzoselenazole nucleus, 5 photographic light-sensitive material having a photographic silver halide emulsion layer containing the dye gives less color stain after development. Also, in the case of using the aforesaid pseudocyanine dye, the reduction in spectrally sensitized sensitivity caused by the use of a color coupler is considerably less. However, the use of said pseudocyanine dye is accompanied with the disadvantage that the dye is diffused into adjacent emulsion layers to spectrally sensitize said emulsion layers owing to the poor adsorption power of the dye to silver halide. On the other hand, when the pseudocyanine dye 10 mentioned above is used together with the sensitizing dye represented by general formula I, the spectrally sensitized sensitivity obtained by supersensitization is markedly increased, the harmful reduction of sensitivity caused by the presence of a color coupler together with the pseudocyanine dye can be 15 completely prevented, and also the formation of color stain is reduced.

When the sensitizing dye represented by general formula II is used together with the sensitizing dye represented by 20 general formula I, no harmful inhibiting action in development by the dyes occurs and, to the contrary, the development tends to be promoted, each of which are particular advantages of the present invention.

The sensitivity in the spectrally sensitive region of from 30 500 to 530  $\mu\mu$  obtained by the use of the combination of the sensitizing dye represented by general formula I and the sensitizing dye represented by general formula II is higher than the sensitivity in that region obtained by the method disclosed in Japanese Pat. Publication No. 4936/68 mentioned above but, 35 strictly speaking, is still not as great as desired. This difficulty can be overcome by further adding at least one compound represented by general formula III.

The sensitizing dyes and, if necessary, the compound used 40 in the present invention, may be dissolved in a water-miscible organic solvent such as methanol, ethanol, alkalified ethanol, acidified methanol, acetone, or pyridine and they may be added to a photographic emulsion either as a mixture or separately. The amount of the additive is varied according to 45 the kind of the silver halide emulsion to be employed but is preferably from  $1 \times 10^{-6}$  mole to  $1 \times 10^{-4}$  mole per 100 g. of the silver halide emulsion. The order of addition of these additives and the proportions may be varied according to the intended purpose.

In general, the ratio of the cyanine dye represented by 50 general formula II to the cyanine dye represented by the general formula I may be from one-tenth to 10, the ratio of the cyanine dye represented by the general formula III to the cyanine dye represented by the general formula I may be from one-tenth to 10. As the photographic silver halide emulsion used in the present invention, there may be mentioned silver chloride emulsion, silver chlorobromide emulsion, silver bromide emulsion, silver iodobromide emulsion and the like. The photographic emulsion of this invention may further contain, aside from the sensitizing dyes of the present invention and, if necessary, the compound of general formula III, such additives as a stabilizer, an antifoggant, a hardening agent, a wetting agent, a plasticizer, and the like. In particular, in the case of preparing a coupler incorporated type of color photographic light-sensitive material, a magenta coupler may be incorporated in the silver halide emulsion containing the aforesaid additives.

The photographic silver halide emulsion of this invention, prepared by the above-mentioned procedures, may be applied 70 to a suitable support such as a cellulose derivative film, a baryta-coated paper, a glass plate, a polyethylene terephthalate film and the like.

Examples of the sensitizing dyes and the compound of formula III used in the present invention are shown below, although the invention is not limited only to those shown.

### Sensitizing dyes represented by general formula I:



### Sensitizing dyes represented by general formula II:



### Compound represented by general formula III:



The sensitizing dyes represented by general formula I may be prepared by the methods described in, for instance, the specifications of U.S. Pat. No. 2,912,329 and Belgian Pat. No. 697,245.

30 Typical examples of preparing the sensitizing dyes represented by general formula II are briefly shown below.

### 1. Preparation of dye (II A):

To a mixture of 100 ml. of ethanol and 6 ml. of triethylamine were added 1 g. of 1-ethyl-2-ethylmercapto-6-methyl-quinolinium p-toluenesulfonate and 1 g. of anhydro 5-hydroxy-2,5-dimethyl-3-( $\gamma$ -sulfopropyl)benzothiazolium hydroxide and the mixture was refluxed by heating for 1 hour to cause the reaction. The crystals thus precipitated were filtered, washed with water, and recrystallized from a mixed solvent of methanol and chloroform to provide crystals of the dye (II A) having a melting point higher than 300°C. and a

λ MeOH

45 of 506

Dyes (II B), (II C), (II D), and (II E) can be also prepared by the above method.

2. the compounds represented by general formula III can be prepared by the following manner.

## 2. Preparation of compound (III A):

In 70 ml. of acetone was suspended 4.7 g. of 2-( $\beta$ -anilinovinyl)-5,6-dichloro-1,3-diethylbenzimidazolium iodide and to the suspension was added dropwise a solution of 2 g. of sodium hydroxide in 25 ml. of water with stirring at room temperature. After 20 minutes, a large amount of water was added to the solution prepared. The crystals thus precipitated were filtered, washed with water, and recrystallized from ligroin to provide 1.2 g. of crystals of compound (III A) having a melting point of 151°C. and

λ MeOH

of 384  $\mu\mu$

65 Other compounds, e.g., (III B) and (III C) can be prepared by the above procedure.

The following examples further illustrate the present invention.

70

### EXAMPLE 1

In a beaker was melted 100 g. of a conventionally prepared gelatino silver iodobromide emulsion (AgI 6.0 mole percent) and, after adding to the emulsion a methanol solution of the sensitizing dye or methanol solutions of the sensitizing dyes,

the system was stirred for 15 minutes at 40°C. Then, a hardening agent was added to the emulsion and thereafter the emulsion was immediately applied to a film support followed by drying to provide a green-sensitive photographic silver halide light sensitive material.

The film was cut into strips and the same strip was exposed to yellow light through Fuji Filter 012 (a yellow filter made by Fuji Photo Film Co.) using an optical wedge and a sensitometer, subjected to black and white development, and then fixed to provide a black and white negative image.

By measuring the density of the black and white negative image thus obtained, the relative green sensitivity was then obtained.

On the other hand, an unexposed sample strip obtained as above was subjected to a spectral exposure by means of a reflection type grating spectroscope and then subjected to black and white development. By measuring the density of the image, a distribution curve of spectral sensitization was obtained.

These results are shown in table 1 together with the sensitizing dyes and the amounts thereof employed. The black and white development was conducted for 10 minutes at 20°C. in the developer having the following composition.

Black and white developer

|                                        |  |       |  |  |
|----------------------------------------|--|-------|--|--|
| N-methyl-p-aminophenol sulfate         |  |       |  |  |
| Sodium sulfite                         |  | 4 g.  |  |  |
| Hydroquinone                           |  | 50 g. |  |  |
| Sodium carbonate (monohydrate)         |  | 5 g.  |  |  |
| Potassium bromide                      |  | 40 g. |  |  |
| Potassium thiocyanate                  |  | 5 g.  |  |  |
| Potassium iodide (0.1% soln.)          |  | 1 g.  |  |  |
| Water to make 1,000 ml. (pH 10.2±0.1). |  | 5 ml. |  |  |

TABLE 1

| (A)                     | (B)                      | (C)  | (D)  | (E)     |
|-------------------------|--------------------------|------|------|---------|
| (IA) $4 \times 10^{-4}$ |                          |      |      |         |
| Mole, 1 ml.             | —                        | 70   | 0.08 | 563     |
| 2 ml.                   | —                        | 79   | 0.10 | 563     |
| —                       | (IIA) $1 \times 10^{-3}$ |      |      |         |
| mole, 2 ml.             | 100                      | 0.15 | 5558 |         |
| —                       | 4 ml.                    | 126  | 0.20 | 558     |
| 2 ml.                   | 4 ml.                    | 159  | 0.15 | 550-560 |
| (IB) $4 \times 10^{-4}$ |                          |      |      |         |
| mole, 1 ml.             | —                        | 40   | 0.13 | 564     |
| 2 ml.                   | —                        | 56   | 0.17 | 564     |
| 4 ml.                   | —                        | 48   | 0.19 | 565     |
| (IB) 1 ml.              | (IIA) $1 \times 10^{-3}$ |      |      |         |
| mole, 4 ml.             | 152                      | 0.22 | 560  |         |
| 2 ml.                   | 4 ml.                    | 152  | 0.22 | 560     |
| (IC) $4 \times 10^{-4}$ |                          |      |      |         |
| mole, 1 ml.             | —                        | 28   | 0.14 | 570     |
| 2 ml.                   | —                        | 20   | 0.16 | 570     |
| 4 ml.                   | —                        | 14   | 0.16 | 571     |
| 2 ml.                   | (IID) $1 \times 10^{-3}$ |      |      |         |
| 2 ml.                   | 4 ml.                    | 141  | 0.16 | 550-570 |
| 2 ml.                   | 4 ml.                    | 160  | 0.17 | 550-570 |
| —                       | 2 ml.                    | 80   | 0.13 | 570     |
| —                       | 4 ml.                    | 100  | 0.17 | 570     |
| —                       | 8 ml.                    | 89   | 0.21 | 570     |

Note: (A) In order, the kind of the sensitizing dye represented by general formula I, the concentration of the dye, and the addition amount thereof; (B) In order, the kind of the sensitizing dye represented by general formula II, the concentration of the dye, and the addition amount thereof; (C) Relative sensitivity; (D) Fog; and (E) Maximum sensitized wave length in  $\mu$ .

From the above results, it was clear that by the combination of the two kinds of the sensitizing dyes represented by general formulas I and II, respectively, a high supersensitization was obtained without increasing the formation of fog to any harmful extent.

EXAMPLE 2

In a beaker was melted 100 g. of a conventionally prepared gelatino silver iodobromide emulsion (AgI 4.0 mole percent) and, after adding to the emulsion a methanol solution of the sensitizing dye or methanol solutions of the sensitizing dyes shown in table 2, the system was stirred for 15 minutes at 35°C. Then 20 ml. of a 5 percent alkaline solution of a magenta coupler having the following structure was added to the emulsion with stirring and the system was neutralized by the addition of citric acid.



A hardening agent was added to the emulsion and thereafter the emulsion was immediately applied to a film support followed by drying to provide a green-sensitive color photographic light-sensitive material.

The light-sensitive film was cut into strips and the sample strip was subjected to a yellow exposure by means of a sensitometer. The sample thus exposed was subjected to a color development for 10 minutes at 20°C. in a color developer, containing as a color developing agent at N,N'-diethylamino-p-aminobenzoic derivative, having the following composition;

|    |                                          |                                             |        |
|----|------------------------------------------|---------------------------------------------|--------|
| 30 | Color developer                          | N,N'-diethylamino-p-aminobenzoic derivative | 2.0 g. |
|    | nitrate                                  |                                             |        |
|    | Sodium sulfite                           |                                             | 2.0 g. |
|    | Sodium carbonate (monohydrate)           | 50.0 g.                                     |        |
|    | Hydroxylamine hydrochloride              | 1.5 g.                                      |        |
|    | Potassium bromide                        | 1.0 g.                                      |        |
|    | Water to make 1,000 ml.<br>(pH 10.8±0.1) |                                             |        |

The sample was then subjected to first fixing, bleaching and second fixing to provide a magenta image. By measuring the density of the magenta image using a green light, a relative green sensitivity was obtained. The results are shown in table 2.

TABLE 2

| (A)                     | (B)                       | (C)  | (D)     | (E)     |
|-------------------------|---------------------------|------|---------|---------|
| (ID) $4 \times 10^{-4}$ |                           |      |         |         |
| mole, 1 ml.             | —                         | 71   | 0.08    | 580     |
| 2 ml.                   | —                         | 100  | 0.10    | 583     |
| 4 ml.                   | —                         | 110  | 0.12    | 583     |
| 2 ml.                   | (IIIC) $1 \times 10^{-3}$ |      |         |         |
| mole, 2 ml.             | 158                       | 0.12 | 578     |         |
| 2 ml.                   | 4 ml.                     | 195  | 0.13    | 576     |
| 2 ml.                   | 8 ml.                     | 188  | 0.14    | 540-570 |
| —                       | 2 ml.                     | 66   | 0.08    | 560     |
| —                       | 4 ml.                     | 71   | 0.13    | 562     |
| —                       | 8 ml.                     | 98   | 0.18    | 562     |
| (ID) $4 \times 10^{-4}$ | (IIB) $1 \times 10^{-3}$  |      |         |         |
| mole, 2 ml.             | 42                        | 0.10 | 560     |         |
| 2 ml.                   | 4 ml.                     | 166  | 0.11    | 550-560 |
| 2 ml.                   | 8 ml.                     | 200  | 0.13    | 545-560 |
| —                       | 2 ml.                     | 79   | 0.08    | 550     |
| —                       | 4 ml.                     | 109  | 0.09    | 550     |
| —                       | 8 ml.                     | 129  | 0.10    | 550     |
| (ID) $4 \times 10^{-4}$ | (IIA) $1 \times 10^{-3}$  |      |         |         |
| mole, 2 ml.             | 200                       | 0.22 | 550-578 |         |
| (ID) 2 ml.              | (IIA) 4 ml.               | 250  | 0.25    | 550-578 |
| 2 ml.                   | 8 ml.                     | 290  | 0.30    | 545-575 |
| —                       | 2 ml.                     | 141  | 0.18    | 562     |
| —                       | 4 ml.                     | 166  | 0.25    | 562     |
| —                       | 8 ml.                     | 178  | 0.32    | 562     |

Note: (A), (B), (C), (D), and (F) have the same meanings as those in table 1.

The above procedure was followed except for the addition of a compound represented by the general formula III. The results are shown below:

TABLE 3

| (A)                           | (B)                             | (C)                                   | (D) | (E)  | (F)     |
|-------------------------------|---------------------------------|---------------------------------------|-----|------|---------|
| (IB) $4 \times 10^{-4}$ mole: | (IIIC) $1 \times 10^{-3}$ mole: |                                       |     |      |         |
| 2 ml.                         | 4 ml.                           |                                       | 200 | 0.16 | 562     |
| 2 ml.                         | 4 ml.                           | (IIIA) $1 \times 10^{-3}$ mole, 2 ml. | 235 | 0.15 | 560     |
| (ID) $4 \times 10^{-4}$ mole: | (IIIA) $1 \times 10^{-3}$ mole: |                                       |     |      |         |
| 1 ml.                         | 4 ml.                           |                                       | 250 | 0.17 | 560     |
| 2 ml.                         | 4 ml.                           | (IIIB) $1 \times 10^{-3}$ mole, 2 ml. | 250 | 0.16 | 550-578 |
| 2 ml.                         | 4 ml.                           |                                       | 282 | 0.15 | 540-560 |

Note: (A) In order, the sensitizing dye represented by general formula I, concentration of the dye, and addition amount thereof; (B) In order, the sensitizing dye represented by general formula II, the concentration of the dye, and the addition amount thereof; (C) In order, the compound represented by general formula III, the concentration of the dye, and the addition amount thereof; (D) Relative sensitivity; (E) Fog; and (F) The maximum sensitization wave length in  $\mu$ .

What is claimed is:

1. A photographic silver halide emulsion comprising at least one cyanine dye represented by general formula I



wherein  $Z_1$  and  $Z_2$  are each nonmetallic atoms necessary to complete the benzimidazole nucleus;  $R_1$  and  $R_2$  are each selected from the group consisting of an alkyl group, a substituted alkyl group and an allyl group;  $R_3$  and  $R_4$  are each selected from the group consisting of an alkyl group and a substituted alkyl group, at least one of said groups  $R_3$  and  $R_4$  being selected from the group consisting of a sulfo-substituted alkyl group and a carboxy-substituted alkyl group;  $X_1^1$  is an anion, and  $p$  is 1 or 2 and at least one cyanine dye represented by general formula II



wherein  $Z_3$  represents nonmetallic atoms necessary to complete a quinoline nucleus;  $Y$  is selected from the group consisting of a sulfur atom and a selenium atom;  $R_5$  and  $R_6$  are each selected from the group consisting of an alkyl group and a substituted alkyl group, at least one of said groups  $R_5$  and  $R_6$  being selected from the group consisting of a sulfo-substituted alkyl group and a carboxy-substituted alkyl group;  $A$  is selected from the group consisting of a hydrogen atom, an alkyl group having one to four carbon atoms and a halogen atom;  $X_2^1$  is an anion and  $q$  is 1 or 2.

2. The photographic silver halide emulsion of claim 1 wherein said benzimidazolenucleus in general formula I is substituted by at least one member selected from the group consisting of a halogen atom, a cyano group, a trichloromethyl group, an alkylaminosulfonyl group and an acetyl group.

3. The photographic silver halide emulsion of claim 1 wherein said quinoline nucleus in general formula II is substituted by at least one member selected from the group consisting of a methyl group, an ethyl group, a hydroxyl group, an alkoxy group and a halogen atom.

4. The photographic silver halide emulsion of claim 1 wherein said sulfo-substituted alkyl group represented by  $R_3$  or  $R_4$  in general formula I and  $R_5$  or  $R_6$  in general formula II is selected from the group consisting of a  $\beta$ -sulfoethyl group, a  $\gamma$ -sulfopropyl group, a  $\gamma$ -sulfobutyl group, a  $\delta$ -sulfobutyl group, a 2-hydroxy-1-sulfopropyl group, a 2-(3-sulfopropoxy)ethyl group, and a 2-[2-(3-sulfopropoxy)ethoxy]ethyl group.

5. The photographic silver halide emulsion of claim 1 wherein said carboxy-substituted alkyl group represented by  $R_3$  or  $R_4$  in general formula I and  $R_5$  and  $R_6$  in general formula II is selected from the group consisting of a  $\beta$ -carboxyethyl group, an  $\alpha$ -carboxypropyl group and a 2-(2-carboxy-ethoxy)ethyl group.

6. The photographic silver halide emulsion of claim 1 wherein said silver halide emulsion containing said cyanine dyes is a green-sensitive silver halide emulsion containing a magenta coupler for color photographic light-sensitive material.

7. A color photographic light-sensitive material comprising a support and at least one layer of a photographic silver halide emulsion as set forth in claim 1.

8. A photographic silver halide emulsion as set forth in claim 1 further comprising at least one compound represented by general formula III



wherein  $Z_4$  represents nonmetallic atoms necessary to complete a benzimidazole nucleus;  $Z_5$  is selected from the group consisting of a phenyl group and a substituted phenyl group; and  $R_7$  is selected from the group consisting of an alkyl group and a substituted alkyl group.

9. The photographic silver halide emulsion of claim 8 wherein said silver halide emulsion is a green sensitive silver halide emulsion containing a magenta coupler for color photographic light-sensitive material.

10. A color photographic light-sensitive material comprising a support and at least one layer of a silver halide emulsion as set forth in claim 8.